# EUROPEAN PATENT SPECIFICATION

(11) **EP 2 138 564 B1**
(45) Date of publication and mention of the grant of the patent: **06.11.2013**
(21) Application number: 08159022.6
(22) Date of filing: 25.06.2008
(51) Int. Cl.: C11D 11/02, C11D 11/04, C11D 11/00

(54) **A process for preparing a detergent powder**
Verfahren zur Herstellung von Waschmittelpulver
Procédé de préparation d'une lessive en poudre

(43) Date of publication of application: 30.12.2009
(73) Proprietor: The Procter & Gamble Company, Cincinnati, OH 45202 (US)
(72) Inventor: Tantawy, Hossam Hassan, Morpeth, Northumberland NE61 3JT (GB); Somerville Roberts, Nigel Patrick, Newcastle upon Tyne, NE20 9UJ (GB); Harrogate, Urwin, Choppington, Northumberland NE62 5YF (GB); York, David William, Newcastle upon Tyne, NE20 9TB (GB)
(74) Representative: Howard, Phillip Jan

(56) References cited:
- DE-A1- 10 235 942
- DE-A1- 19 936 613
- US-A- 3 844 969
- US-A- 3 996 149
- US-A- 4 362 640

## Description

### FIELD OF THE INVENTION

The present invention relates to a process for preparing a powder.

### BACKGROUND OF THE INVENTION

There is a recent trend in the laundry detergent industry to produce low-built laundry powders. These are typically produced by a process involving a drying step. However, during conventional drying steps, such as conventional spray-drying, the low-built powders produced by these processes have a poor stability profile. This is exacerbated when a significant amount of silicate salt is present in the spray-dried powder. The Inventors have overcome this problem by incorporating a volatile compound into the detergent slurry making process, and carefully controlling the pressure during the process such that low-built, anionic detersive surfactant-containing powders are produced that have good stability profiles.

DE-A-10235942, DE-A-19936613, US-A-3996149 and US-A-3844969 relate to processes for making compositions of matter.

### SUMMARY OF THE INVENTION

The present invention relates to a process as defined by claim 1.

### DETAILED DESCRIPTION OF THE INVENTION

### Spray-drying process

The process comprises the steps of: (a) forming a slurry that comprises a volatile compound; and (b) spraying the slurry through a nozzle into a drying apparatus; and (c) drying the slurry to form a powder. The slurry enters the nozzle at one of two of the below described conditions.
(I) At the temperature at which the slurry enters the nozzle, the slurry is at a pressure that is equal to or greater than the vapour pressure of the volatile component. In addition, the slurry enters the nozzle at a temperature such that the vapour pressure of the volatile compound is above the pressure in the drying apparatus.
(II) The volatile component is in supercritical form when the slurry enters the nozzle. In addition, when the volatile component is in supercritical form when the slurry enters the nozzle, the conditions in the drying apparatus are such that when the volatile component enters the drying apparatus, at least a portion, preferably essentially all of the volatile component is in gaseous form.

In step (b) the slurry is sprayed at a temperature of below 125°C, or below 100°C, or below 90°C, or below 80°C, or below 70°C, or even below 60°C into the drying apparatus.

Preferably, the powder is in spray-dried form, and wherein the drying apparatus is a spray-drying tower. Alternatively, the drying apparatus is a powder mixing apparatus and/or a fluid bed dryer.

Preferably, the powder produced in step (c) is contacted with non-ionic detersive surfactant.

### Powder

The powder comprises (i) anionic detersive surfactant; (ii) from 0wt% to 10wt% zeolite builder; (iii) from 0wt% to 10wt% phosphate builder; and (iv) from 0wt% to 15wt% silicate salt. Preferably, the powder comprises from 3wt% to 15wt% silicate salt. The powder preferably comprises a carbonate salt. The powder may comprise detergent adjunct ingredients. The powder is preferably in spray-dried form.

### Slurry

Typically, the slurry comprises water; the slurry is typically an aqueous slurry. The slurry comprises a volatile component. This is preferably formed by injection of the volatile component into the slurry under pressure. Alternatively, it could be formed by the in-situ formation of the volatile component in the slurry, e.g. by the neutralization of an acid anionic surfactant precursor with a carbonate salt. The volatile component may even be formed by the thermal decomposition of a salt, e.g. sodium bicarbonate.

### Anionic detersive surfactant

The anionic detersive surfactant preferably comprises alkyl benzene sulphonate. Preferably the anionic detersive surfactant comprises at least 50%, preferably at least 55%, or at least 60%, or at least 65%, or at least 70%, or even at least 75%, by weight of the anionic detersive surfactant, of alkyl benzene sulphonate. Preferably the alkyl benzene sulphonate is a linear or branched, substituted or unsubstituted, C₈₋₁₈ alkyl benzene sulphonate. This is the optimal level of the C₈₋₁₈ alkyl benzene sulphonate to provide a good cleaning performance. The C₈₋₁₈ alkyl benzene sulphonate can be a modified alkylbenzene sulphonate (MLAS) as described in more detail in WO 99/05243, WO 99/05242, WO 99/05244, WO 99/05082, WO 99/05084, WO 99/05241, WO 99/07656, WO 00/23549, and WO 00/23548. Highly preferred C₈₋₁₈ alkyl benzene sulphonates are linear C₁₀₋₁₃ alkylbenzene sulphonates. Especially preferred are linear C₁₀₋₁₃ alkylbenzene sulphonates that are obtainable, preferably obtained, by sulphonating commercially available linear alkyl benzenes (LAB); suitable LAB include low 2-phenyl LAB, such as those supplied by Sasol under the tradename Isocher^{®} or those supplied by Petresa under the tradename Petrelab^{®}, other suitable LAB include high 2-phenyl LAB, such as those supplied by Sasol under the tradename Hyblene^{®}.

The anionic detersive surfactant may preferably comprise other anionic detersive surfactants. A preferred adjunct anionic detersive surfactant is a non-alkoxylated anionic detersive surfactant. The non-alkoxylated anionic detersive surfactant can be an alkyl sulphate, an alkyl phosphate, an alkyl phosphonate, an alkyl carboxylate or any mixture thereof. The non-alkoxylated anionic surfactant can be selected from the group consisting of; C₁₀-C₂₀ primary, branched-chain, linear-chain and random-chain alkyl sulphates (AS), typically having the following formula:

CH₃(CH₂)ₓCH₂-OSO₃⁻M⁺

wherein, M is hydrogen or a cation which provides charge neutrality, preferred cations are sodium and ammonium cations, wherein x is an integer of at least 7, preferably at least 9; C₁₀-C₁₈ secondary (2,3) alkyl sulphates, typically having the following formulae: wherein, M is hydrogen or a cation which provides charge neutrality, preferred cations include sodium and ammonium cations, wherein x is an integer of at least 7, preferably at least 9, y is an integer of at least 8, preferably at least 9; C₁₀-C₁₈ alkyl carboxylates; mid-chain branched alkyl sulphates as described in more detail in US 6,020,303 and US 6,060,443; methyl ester sulphonate (MES); alpha-olefin sulphonate (AOS); and mixtures thereof.

Another preferred anionic detersive surfactant is an alkoxylated anionic detersive surfactant. The presence of an alkoxylated anionic detersive surfactant in the spray-dried powder provides good greasy soil cleaning performance, gives a good sudsing profile, and improves the hardness tolerance of the anionic detersive surfactant system. It may be preferred for the anionic detersive surfactant to comprise from 1% to 50%, or from 5%, or from 10%, or from 15%, or from 20%, and to 45%, or to 40%, or to 35%, or to 30%, by weight of the anionic detersive surfactant system, of an alkoxylated anionic detersive surfactant.

Preferably, the alkoxylated anionic detersive surfactant is a linear or branched, substituted or unsubstituted C₁₂₋₁₈ alkyl alkoxylated sulphate having an average degree of alkoxylation of from 1 to 30, preferably from 1 to 10. Preferably, the alkoxylated anionic detersive surfactant is a linear or branched, substituted or unsubstituted C₁₂₋₁₈ alkyl ethoxylated sulphate having an average degree of ethoxylation of from 1 to 10. Most preferably, the alkoxylated anionic detersive surfactant is a linear unsubstituted C₁₂₋₁₈ alkyl ethoxylated sulphate having an average degree of ethoxylation of from 3 to 7.

The alkoxylated anionic detersive surfactant, when present with an alkyl benzene sulphonate may also increase the activity of the alkyl benzene sulphonate by making the alkyl benzene sulphonate less likely to precipitate out of solution in the presence of free calcium cations. Preferably, the weight ratio of the alkyl benzene sulphonate to the alkoxylated anionic detersive surfactant is in the range of from 1:1 to less than 5:1, or to less than 3:1, or to less than 1.7:1, or even less than 1.5:1. This ratio gives optimal whiteness maintenance performance combined with a good hardness tolerance profile and a good sudsing profile. However, it may be preferred that the weight ratio of the alkyl benzene sulphonate to the alkoxylated anionic detersive surfactant is greater than 5:1, or greater than 6:1, or greater than 7:1, or even greater than 10:1. This ratio gives optimal greasy soil cleaning performance combined with a good hardness tolerance profile, and a good sudsing profile.

Suitable alkoxylated anionic detersive surfactants are: Texapan LEST™ by Cognis; Cosmacol AES™ by Sasol; BES 151™ by Stephan; Empicol ESC70/U™; and mixtures thereof.

Preferably, the anionic detersive surfactant comprises from 0% to 10%, preferably to 8%, or to 6%, or to 4%, or to 2%, or even to 1%, by weight of the anionic detersive surfactant, of unsaturated anionic detersive surfactants such as alpha-olefin sulphonate. Preferably the anionic detersive surfactant is essentially free of unsaturated anionic detersive surfactants such as alpha-olefin sulphonate. By "essentially free of" it is typically meant "comprises no deliberately added". Without wishing to be bound by theory, it is believed that these levels of unsaturated anionic detersive surfactants such as alpha-olefin sulphonate ensure that the anionic detersive surfactant is bleach compatible.

Preferably, the anionic detersive surfactant comprises from 0% to 10%, preferably to 8%, or to 6%, or to 4%, or to 2%, or even to 1%, by weight of alkyl sulphate. Preferably the anionic detersive surfactant is essentially free of alkyl sulphate. Without wishing to be bound by theory, it is believed that these levels of alkyl sulphate ensure that the anionic detersive surfactant is hardness tolerant.

### Volatile compound

The volatile component is water.

The volatile component may be in supercritical form. It may be especially preferred for the volatile component to be in supercritical form when it enters the nozzles.

Typically, the volatile component is in liquid form.

### Zeolite builder

The powder typically comprises from 0% to 10wt% zeolite builder, preferably to 9wt%, or to 8wt%, or to 7wt%,or to 6wt%, or to 5wt%, or to 4wt%, or to 3wt%, or to 2wt%, or to 1wt%, or to less than 1% by weight of the powder, of zeolite builder. It may even be preferred for the powder to be essentially free from zeolite builder. By essentially free from zeolite builder it is typically meant that the powder comprises no deliberately added zeolite builder. This is especially preferred if it is desirable for the powder to be very highly soluble, to minimize the amount of water-insoluble residues (for example, which may deposit on fabric surfaces), and also when it is highly desirable to have transparent wash liquor. Zeolite builders include zeolite A, zeolite X, zeolite P and zeolite MAP.

### Phosphate builder

The powder typically comprises from 0% to 10wt% phosphate builder, preferably to 9wt%, or to 8wt%, or to 7wt%,or to 6wt%, or to 5wt%, or to 4wt%, or to 3wt%, or to 2wt%, or to 1wt%, or to less than 1% by weight of the powder, of phosphate builder. It may even be preferred for the powder to be essentially free from phosphate builder. By essentially free from phosphate builder it is typically meant that the powder comprises no deliberately added phosphate builder. This is especially preferred if it is desirable for the powder to have a very good environmental profile. Phosphate builders include sodium tripolyphosphate.

### Silicate salt

The powder optionally comprises from 0% to 20wt% silicate salt, preferably from 1wt%, or from 2wt%, or from 3wt%, and preferably to 15wt%, or to 10wt%, or even to 5% silicate salt. Silicate salts include amorphous silicates and crystalline layered silicates (e.g. SKS-6). A preferred silicate salt is sodium silicate.

### Carbonate salt

The powder typically comprises carbonate salt, typically from 1% to 50%, or from 5% to 25% or from 10% to 20%, by weight of the powder, of carbonate salt. A preferred carbonate salt is sodium carbonate and/or sodium bicarbonate. A highly preferred carbonate salt is sodium carbonate. Preferably, the powder may comprise from 10% to 40%, by weight of the powder, of sodium carbonate. However, it may also be preferred for the powder to comprise from 2% to 8%, by weight of the powder, of sodium bicarbonate. Sodium bicarbonate at these levels provides good alkalinity whilst minimizing the risk of surfactant gelling which may occur in surfactant-carbonate systems. If the spray-dried powder comprises sodium carbonate and zeolite, then preferably the weight ratio of sodium carbonate to zeolite is at least 15:1.

High levels of carbonate improve the cleaning performance of the composition by increasing the pH of the wash liquor. This increased alkalinity: improves the performance of the bleach, if present; increases the tendency of soils to hydrolyse, which facilitates their removal from the fabric; and also increases the rate, and degree, of ionization of the soils to be cleaned (n.b. ionized soils are more soluble and easier to remove from the fabrics during the washing stage of the laundering process). In addition, high carbonate levels improve the flowability of the powder.

### Adjunct detergent ingredients

Suitable adjunct detergent ingredients include: detersive surfactants such as anionic detersive surfactants, nonionic detersive surfactants, cationic detersive surfactants, zwitterionic detersive surfactants, amphoteric detersive surfactants; preferred nonionic detersive surfactants are C₈₋₁₈ alkyl alkoxylated alcohols having an average degree of alkoxylation of from 1 to 20, preferably from 3 to 10, most preferred are C₁₂₋₁₈ alkyl ethoxylated alcohols having an average degree of alkoxylation of from 3 to 10; preferred cationic detersive surfactants are mono-C₆₋₁₈ alkyl mono-hydroxyethyl di-methyl quaternary ammonium chlorides, more preferred are mono-C₈₋₁₀ alkyl mono-hydroxyethyl di-methyl quaternary ammonium chloride, mono-C₁₀₋₁₂ alkyl mono-hydroxyethyl di-methyl quaternary ammonium chloride and mono-C₁₀ alkyl mono-hydroxyethyl di-methyl quaternary ammonium chloride; source of peroxygen such as percarbonate salts and/or perborate salts, preferred is sodium percarbonate, the source of peroxygen is preferably at least partially coated, preferably completely coated, by a coating ingredient such as a carbonate salt, a sulphate salt, a silicate salt, borosilicate, or mixtures, including mixed salts, thereof; bleach activator such as tetraacetyl ethylene diamine, oxybenzene sulphonate bleach activators such as nonanoyl oxybenzene sulphonate, caprolactam bleach activators, imide bleach activators such as N-nonanoyl-N-methyl acetamide, preformed peracids such as N,N-pthaloylamino peroxycaproic acid, nonylamido peroxyadipic acid or dibenzoyl peroxide; enzymes such as amylases, carbohydrases, cellulases, laccases, lipases, oxidases, peroxidases, proteases, pectate lyases and mannanases; suds suppressing systems such as silicone based suds suppressors; fluorescent whitening agents; photobleach; filler salts such as sulphate salts, preferably sodium sulphate; fabric-softening agents such as clay, silicone and/or quaternary ammonium compounds; flocculants such as polyethylene oxide; dye transfer inhibitors such as polyvinylpyrrolidone, poly 4-vinylpyridine N-oxide and/or co-polymer of vinylpyrrolidone and vinylimidazole; fabric integrity components such as hydrophobically modified cellulose and oligomers produced by the condensation of imidazole and epichlorhydrin; soil dispersants and soil anti-redeposition aids such as alkoxylated polyamines and ethoxylated ethyleneimine polymers; anti-redeposition components such as carboxymethyl cellulose and polyesters; perfumes; sulphamic acid or salts thereof; citric acid or salts thereof; and dyes such as orange dye, blue dye, green dye, purple dye, pink dye, or any mixture thereof.

### Further embodiment

In a further embodiment, the present invention provides a process for preparing a powder comprising: (i) anionic detersive surfactant; (ii) from 0wt% to 10wt% zeolite builder; (iii) from 0wt% to 10wt% phosphate builder; and (iv) from 0wt% to 15wt% silicate salt; wherein the process comprises the steps of: (a) contacting an aqueous slurry with carbon dioxide to form a mixture; and (b) spraying the mixture through a nozzle into a drying apparatus; and (c) drying the slurry to form a powder.

Preferably the carbon dioxide is formed by the neutralization of an acid anionic surfactant precursor with a carbonate salt and/or thermal decomposition of a carbonate salt, typically a bicarbonate salt, most preferably sodium bicarbonate.

### EXAMPLES

### Example 1. A particulate laundry detergent composition and process of making it. (reference example)

### Aqueous slurry composition.

| **Component** | **Aqueous slurry (parts)** |
|---|---|
| Ethylenediamine disuccinic acid | 0.35 |
| Magnesium sulphate | 0.72 |
| Sodium silicate | 6.45 |
| Linear alkyl benzene sulphonate | 11.92 |
| Hydroxyethane di(methylene phosphonic acid) | 0.32 |
| Sodium carbonate | 4.32 |
| Sodium sulphate | 47.49 |
| Water | 25.89 |
| Miscellaneous | 0.42 |
| **Total Parts** | **100.00** |

### Preparation of a spray-dried powder.

An aqueous slurry having the composition as described above is prepared having a moisture content of 25.89%. The aqueous slurry is heated to 72°C and pumped into a low pressure line (having a pressure of 5x10⁵ Pa), and then into a high pressure line (having an exit pressure of 8x10⁶ Pa). Liquid CO₂ is injected into the high pressure line. The resultant slurry is then sprayed at pressure of 8x10⁶ Pa and at a temperature of 65°C through a nozzle into a counter-current spray-drying tower with an air inlet temperature of from 270°C to 300°C and at a pressure of less than 1x10⁵ Pa. The aqueous slurry is atomised and the atomised slurry is dried to produce a solid mixture, which is then cooled and sieved to remove oversize material (>1.8mm) to form a spray-dried powder, which is free-flowing. Fine material (<0.15mm) is elutriated with the exhaust air in the spray-drying tower and collected in a post tower containment system. The spray-dried powder has a moisture content of 2.5wt%, a bulk density of 427g/l and a particle size distribution such that 95.2wt% of the spray-dried powder has a particle size of from 150 to 710 micrometers. The composition of the spray-dried powder is given below.

### Spray-dried powder composition.

| **Component** | **%w/w Spray-dried powder** |
|---|---|
| Magnesium sulphate | 0.96 |
| Sodium silicate | 8.62 |
| Linear alkyl benzene sulphonate | 15.92 |
| Hydroxyethane di(methylene phosphonic acid) | 0.43 |
| Sodium carbonate | 5.77 |
| Sodium sulphate | 63.43 |
| Water | 2.5 |
| Miscellaneous | 0.55 |
| **Total Parts** | **100.00** |

## Claims

1. A process for preparing a powder comprising:
(i) anionic detersive surfactant;
(ii) from 0wt% to 10wt% zeolite builder;
(iii) from 0wt% to 10wt% phosphate builder; and
(iv) from 0wt% to 15wt% silicate salt;
wherein the process comprises the steps of:
(a) forming a slurry that comprises a volatile compound; and
(b) spraying the slurry through a nozzle into a drying apparatus; and
(c) drying the slurry to form a powder,
wherein the slurry enters the nozzle at conditions such that either:
(I) at the temperature at which the slurry enters the nozzle, the slurry is at a pressure that is equal to or greater than the vapour pressure of the volatile component, and wherein, the slurry enters the nozzle at a temperature such that the vapour pressure of the volatile compound is above the pressure in the drying apparatus; or
(II) the volatile component is in supercritical form when the slurry enters the nozzle, and
wherein, the conditions in the drying apparatus are such that when the volatile component enters the drying apparatus, at least a portion of the volatile component is in gaseous form, wherein the volatile component is water, and wherein in step (b) the slurry is sprayed at a temperature of below 125°C.

2. A process according to any preceding claim, wherein in step (b) the mixture is sprayed at a temperature of below 100°C into the drying apparatus.

3. process according to any preceding claim, wherein the powder is in spray-dried form, and
wherein the drying apparatus is a spray-drying tower.

4. A process according to any preceding claim, wherein the drying apparatus is a powder mixing apparatus.

5. A process according to any preceding claim, wherein the drying apparatus is a fluid bed dryer.

6. A process according to any preceding claim, wherein the powder produced in step (c) is contacted with non-ionic detersive surfactant.

## Patentansprüche

1. Verfahren zum Herstellen eines Pulvers, umfassend:
(i) ein anionisches Reinigungstensid,
(ii) zu 0 Gew.-% bis 10 Gew.-% Zeolithbuilder,
(iii) zu 0 Gew.-% bis 10 Gew.-% Phosphatbuilder und
(iv) zu 0 Gew-% bis 15 Gew-% Silikatsalz,
wobei das Verfahren die folgenden Schritte umfasst:
(a) Ausbilden einer Schlämme, die eine flüchtige Verbindung umfasst, und
(b) Sprühen der Schlämme durch eine Düse in eine Trocknungsvorrichtung und
(c) Trocknen der Schlämme, um ein Pulver auszubilden,
wobei die Schlämme unter solchen Bedingungen in die Düse gelangt, dass entweder:
(I) bei der Temperatur, bei der die Schlämme in die Düse gelangt, die Schlämme einen Druck aufweist, der bei oder über dem Dampfdruck der flüchtigen Komponente liegt, und wobei die Schlämme bei einer solchen Temperatur in die Düse gelangt, dass der Dampfdruck der flüchtigen Verbindung über dem Druck in der Trocknungsvorrichtung liegt, oder
(II) die flüchtige Komponente in superkritischer Form vorliegt, wenn die Schlämme in die Düse gelangt, und wobei die Bedingungen in der Trocknungsvorrichtung so sind, dass dann, wenn die flüchtige Komponente in die Trocknungsvorrichtung gelangt, zumindest ein Teil der flüchtigen Komponente in Gasform vorliegt, wobei die flüchtige Komponente Wasser ist, und wobei in Schritt (b) die Schlämme bei einer Temperatur von unter 125 °C versprüht wird.

2. Verfahren nach einem der vorstehenden Ansprüche, wobei in Schritt (b) die Mischung bei einer Temperatur von unter 100 °C in die Trocknungsvorrichtung gesprüht wird.

3. Verfahren nach einem der vorstehenden Ansprüche, wobei das Pulver in sprühgetrockneter Form vorliegt, und wobei die Trocknungsvorrichtung ein Sprühtrocknungsturm ist.

4. Verfahren nach einem der vorstehenden Ansprüche, wobei die Trocknungsvorrichtung eine Pulvermischvorrichtung ist.

5. Verfahren nach einem der vorstehenden Ansprüche, wobei die Trocknungsvorrichtung ein Fluidbetttrockner ist.

6. Verfahren nach einem der vorstehenden Ansprüche, wobei das in Schritt (c) erzeugte Pulver mit nicht-ionischem Reinigungstensid in Kontakt gebracht wird.

## Revendications

1. Procédé pour préparer une poudre comprenant :
(i) un agent tensioactif détersif anionique ;
(ii) de 0 % en poids à 10 % en poids d'adjuvant zéolite ;
(iii) de 0 % en poids à 10 % en poids d'adjuvant phosphate ; et
(iv) de 0 % en poids à 15 % en poids de sel de silicate ;
où le procédé comprend les étapes consistant à :
(a) former une bouillie qui comprend un composé volatil ; et
(b) pulvériser la bouillie à travers une buse dans un appareil de séchage ; et
(c) sécher la bouillie de façon à former une poudre,
dans lequel la bouillie pénètre dans la buse à l'une ou l'autre des conditions telles que :
(I) à la température à laquelle la bouillie pénètre dans la buse, la bouillie est à une pression qui est égale ou supérieure à la pression de vapeur du composant volatil, et dans lequel, la bouillie pénètre dans la buse à une température telle que la pression de vapeur du composé volatil est au-dessus de la pression dans l'appareil de séchage ; ou
(II) le composant volatil est sous forme surcritique lorsque la bouillie pénètre dans la buse, et dans lequel, les conditions dans l'appareil de séchage sont telles que lorsque le composant volatil pénètre dans l'appareil de séchage, au moins une partie du composant volatil est sous forme gazeuse, dans lequel le composant volatil est de l'eau, et dans lequel dans l'étape (b) la bouillie est vaporisée à une température inférieure à 125 °C.

2. Procédé selon l'une quelconque des revendications précédentes, dans lequel dans l'étape (b) le mélange est vaporisé à une température inférieure à 100 °C dans l'appareil de séchage.

3. Procédé selon l'une quelconque des revendications précédentes, dans lequel la poudre est sous forme séchée par atomisation, et dans lequel l'appareil de séchage est une tour de séchage par atomisation.

4. Procédé selon l'une quelconque des revendications précédentes, dans lequel l'appareil de séchage est un appareil de mélange de poudre.

5. Procédé selon l'une quelconque des revendications précédentes, dans lequel l'appareil de séchage est un séchoir à lit fluidisé.

6. Procédé selon l'une quelconque des revendications précédentes, dans lequel la poudre produite dans l'étape (c) est mise en contact avec un agent tensioactif détersif non ionique.
